

C. ELLIS.  
PROCESS OF TREATING LEAD.  
APPLICATION FILED JULY 31, 1911.

1,141,177.

Patented June 1, 1915.

Fig. 1.



Fig. 2.



Witnesses:

Sydney M. Spedon.  
Nathaniel L. Foster

Inventor:  
Cathleen Ellis

# UNITED STATES PATENT OFFICE.

CARLETON ELLIS, OF MONTCLAIR, NEW JERSEY, ASSIGNOR TO ELLIS-FOSTER COMPANY, A CORPORATION OF NEW JERSEY.

## PROCESS OF TREATING LEAD.

1,141,177.

Specification of Letters Patent.

Patented June 1, 1915.

Application filed July 31, 1911. Serial No. 641,668.

*To all whom it may concern:*

Be it known that I, CARLETON ELLIS, a citizen of the United States, and a resident of Montclair, in the county of Essex and State of New Jersey, have invented certain new and useful Improvements in Processes of Treating Lead, of which the following is a specification.

This invention relates to a method of 10 comminuting metallic lead or similar metal to form a product especially adapted for preparing pigments such as white lead.

In the so called quick processes for the production of white lead, various means 15 have been employed for reducing the lead to a finely divided state prior to acting upon it with those reagents which bring about its conversion to white lead. Molten lead for example is granulated by pouring it 20 into water or comminuting by means of a jet of steam or air or inert gases, or by forcing through very small orifices so as to produce a fine lead wire.

In this finely divided condition lead is 25 converted into white lead with more or less ease partly depending upon the surface condition of the metal after comminution. Under certain conditions apparently it is possible to cause the surface of the lead particles during the process of comminution to become coated with an oxid which has a catalytic action as regards the subsequent reactions which bring about the conversion 30 to white lead. In many cases however the surface of the lead seemingly becomes coated with a resistant material which protects the lead particles from corrosion during the operation of conversion to white lead so that the process of conversion is greatly 35 retarded and the final product often is not pure white in color but is more or less creamy depending on the amount of the unconverted or partly converted material.

The present invention involves the production of comminuted lead preferably substantially free from superficial oxidation, or in a condition readily susceptible to the action of the reagents employed in the conversion of lead to white lead so that this operation may take place rapidly and completely.

The comminuted lead derived in this manner is of such a character that it is particularly adapted for the manufacture of white lead by those processes employing merely air, moisture and carbon dioxid for the

conversion so that costly reagents such as acetic acid and the like are not necessarily required.

In comminuting the lead it is desirable to have the molten lead brought to a super-molten state *i. e.* to a temperature of 400° or 500° above melting point. Also it is desirable in order to produce a proper comminution or filamentation to eject the lead under considerable pressure. Ordinarily a pressure of 300 to 400 lbs. to the square inch is desirable, and this may be obtained by maintaining a column of molten lead sufficiently high to produce aforesaid pressure. Under such a pressure the lead passing out through the atomizing jets breaks down into very fine particles which are substantially free from that oxidation ordinarily developed by air or steam atomizing jets at this high temperature, and this clean filamentous lead is specially susceptible to the action of air, moisture and the carbon dioxid in the treating tanks. I prefer to conduct the operation so as to obtain the lead in the form of short threads, fibers or filaments. It is also possible to comminute or filament the lead by centrifugal force and for this purpose the molten lead may be fed into a centrifugal at the periphery of which are orifices or nozzles through which the molten lead may pass. Under the combined action of the pressure of the deep column of the molten lead and centrifugal force the lead is ejected from the nozzles in the form of short hairs or filaments which are also readily corroded in the treating tanks.

In the accompanying drawings a melting furnace and atomizer is shown in section.

In Figure 1 the various tanks employed for conversion are shown in elevation. Fig. 2 illustrates the centrifugal atomizer which may be employed in lieu of the angular jet atomizer illustrated in Fig. 1.

The drawings show the various essential features of the apparatus in diagrammatic form.

In the drawings, 1 is a deep pot or receptacle for holding molten lead, to which is attached the melting pot 2. A grate 3 is placed under the melting pot 2, and the waste gases from the fire which is carried on this grate are allowed to pass around the pressure pot 1 in order to maintain the lead at the proper degree of liquidity.

4 and 5 are small round outlets or nozzles

in the lower part of the pressure pot 1, so disposed that their tips nearly meet at a decided angle of impingement.

7 and 8 are rods controlling flow of the metal through the jets 4 and 5.

9 is a receiving tank which ordinarily should be partly filled with water. If desired the tank may be filled with an inert gas in order to avoid traces of oxidation. 10 This tank is provided with the outlet 10 which is arranged for discharge of material into the treating tank 11. The latter may be arranged in the form of a drum or tumbler operating on the journals 12. Means 15 are provided at 13 for the introduction of air or a mixture of air and carbon dioxid. Means are provided at 14 to convey the material from tank 11 into the tank 15 which is similar in arrangement to the tank 11 20 with an inlet 16 for the introduction of carbon dioxid. Means are also provided at 17 for the conveyance of the material from this tank to the driers 18. The tanks 11 and 15 are provided with the gas exits 19 and 25 respectively.

In Fig. 2 a centrifugal means is very diagrammatically shown. This may consist of a drum 19' carrying the nozzles 20' and inlet for the molten lead at 21. Any suitable mechanism may be used for driving this centrifugal.

The operation of the apparatus of Fig. 1 is as follows: Pig lead or other lead material is placed in the melting tank 2, and is brought to a molten state. It overflows into the receptacle 1 and is there raised to a temperature which makes the lead sufficiently liquid to flow readily through the atomizers. When a depth of lead is reached 35 which is sufficient to produce the proper pressure, which as stated should ordinarily be about 300 or 400 lbs. per square inch, the lead is allowed to flow through the atomizers 4 and 5 and when the two streams meet at the point of impingement the lead is reduced to a very finely divided condition and falls into water contained in the tank 9. The lead is then drawn into the tank 11 and treated with air and moisture until more or 40 less hydrated. It may also be treated at this point with carbon dioxid to bring about the carbonation. Sometimes however the lead material is hydrated in the chamber 11, and passed on to the chamber 15 for carbonation. Carbon dioxid is introduced through 45 the pipe 16 and the flow of gas is continued until ordinary hydrated carbonate of lead is produced. The white lead material is then dried in the drying chamber 18. The minute details of the apparatus employed are 50 not here shown and described, but only those figures which are essential to make clear the steps involved in the process.

It will be evident that various modifications may be made in the manner of han-

dling the material, and the present invention contemplates the treatment of the material in a manner which is substantially continuous, or substantially discontinuous. The atomizing jets may be increased in number and 70 several jets may be arranged to direct to the common center or point of impingement, as will be evident from the aforesaid. The comminuted lead may be treated in conveyers instead of in treating tanks if desired so 75 as to give the operation a greater degree of continuity. The lead is preferably maintained as stated at a temperature of 400° to 500° above the melting point, and should be discharged at the atomizers as hereinbefore 80 indicated preferably at a pressure of 300 to 400 lbs. to the square inch, although under certain circumstances even less than this may be used, and in some cases higher pressures 85 are desirable.

While it is not necessary to make use of any chemical reagents such as acetic acid in the conversion of the lead to white lead, such reagents may of course be used if desired, but inasmuch as they add to the cost 90 of the treatment, and as the lead in the particular comminuted or filamentous form derived through this operation is especially susceptible to conversion by air and carbon dioxid in the presence of moisture, such 95 strong chemical reagents need not be employed.

In a second modification of my process the comminuted lead is coated with a very thin layer of catalytic oxid, that is an oxid 100 in a form capable of accelerating, more or less, the subsequent hydration or carbonation reactions.

As stated, the degree of fineness of the filamentous or comminuted lead is a most 105 important consideration. Excessive comminution to a degree double or triple that heretofore practised in the art is one of the first considerations leading to a high grade product. Ordinary impingement of a jet 110 of air or steam and the like has not been carried out in a manner affording a product of the requisite degree of fineness. This may be due to the cooling effect of expansion of the compressed fluid jet. For example, 115 superheated steam under high pressure, suddenly ejected through an orifice and expanded to atmospheric pressure, falls in temperature sometimes many hundred degrees through absorption of heat due to expansion. Hence when the steam contacts with the molten metal it exerts a chilling 120 action which causes coarse granules. In the present invention means are shown for overcoming this defect, the preferred form being 125 the impingement of two or more streams of molten lead against one another at pronounced angle whereby the metal is subdivided to a considerable degree without chilling and the subsequent further commi- 130

nution with a pressure jet. In lieu of initial impingement of the molten metal streams means may be provided for heating the pressure jet after leaving the directing nozzle by 5 immediately passing the ejected gas or steam through a zone of very high temperature, such for example as that afforded by an electric arc formed between electrodes at or near the tip of the directing nozzle.

10 In the drawings a jet 6 is shown positioned near the metal nozzles 4 and 5 arranged to coöperate with the latter in the manner indicated above. In Fig. 2 an annulus (not shown) may be placed around the 15 centrifugal comminutor in such a manner that an annular wall or sheet of steam or air is directed against the issuing material.

In the subsequent treatment of the very finely divided material I prefer to hydrate 20 and carbonate simultaneously as indicated and also to conduct the operation so as to avoid the separation of unchanged lead, but I do not wish to limit myself to this precise procedure as, if for any reason, such as the 25 formation of special pigments and the like

modifications are required involving separation of lead or definite points of hydration or carbonation such changes would not be departing from the spirit of my invention.

30

What I claim is:—

1. In the process of making white lead the step which comprises heating lead to melt same, forcing the molten product in streams into mutual impingement and in exploding 35 the molten spray by a jet of steam.

2. In the process of making white lead, the step which comprises melting lead, forcing the molten metal into two or more streams and in causing these streams to 40 mutually impinge under substantial pressure; whereby the metal is comminuted.

Signed at Chesham, in the county of Cheshire and State of New Hampshire, this 27th day of July, A. D. 1911.

CARLETON ELLIS.

Witnesses:

BIRDELLA M. ELLIS,  
THEODORE ELLIS.